

Oct. 12, 1926.

1,602,553

G. A. RICHTER

## PROCESS OF PRODUCING PULP HIGH IN RESISTANT CELLULOSE

Filed Nov. 11, 1924



Patented Oct. 12, 1926.

1,602,553

# UNITED STATES PATENT OFFICE.

GEORGE A. RICHTER, OF BERLIN, NEW HAMPSHIRE, ASSIGNOR TO BROWN COMPANY, OF BERLIN, NEW HAMPSHIRE, A CORPORATION OF MAINE.

## PROCESS OF PRODUCING PULP HIGH IN RESISTANT CELLULOSE.

Application filed November 11, 1924. Serial No. 749,215.

This invention has relation to the production of cellulose pulp from wood, and has particularly for its object the production of wood pulp, having a high alpha cellulose content. The invention has further for its object to provide a process which is economical and in which certain other advantages are attained as will be subsequently explained in detail. The process which I shall herein describe is practiced in those plants where both sulphite and soda or sulphate pulps are produced.

In accordance with the present invention, the pulp, which is produced by the acid sulphite digestion, is treated with the black liquor resulting from the alkaline digestion, as a result of which results are achieved which have not heretofore been possible.

On the accompanying drawing, I have illustrated conventionally apparatus which may be utilized in the practice of my process, the drawing corresponding to what is known as a flow sheet and being diagrammatic and conventional.

It is my purpose, as previously stated, to utilize a part of the alkaline black liquor resulting from the alkaline digestion of the wood in treating the pulp derived from the wood by the acid-sulphite digestion, for the production of a pulp which has a minimum percentage of nonresistant cellulose,—beta and gamma cellulose,—and a high percentage of resistant or alpha cellulose.

On the drawing, 1 indicates conventionally an acid sulphite digester in which spruce or other suitable wood chips are cooked in an acid sulphite solution of sufficient strength, under conditions of temperature and pressure, until the cellulose fiber is freed from the encrusting or cementitious part of the wood. The strength of the acid solution will depend upon circumstances, but ordinarily I prefer a solution containing, say, 5% free  $\text{SO}_2$  and 1% combined  $\text{SO}_2$ . After the cooking operation is completed, the pulp and the waste liquor are blown into a blow pit indicated at 2, this being the normal operation followed in the acid digestion of wood. In the blow pit the waste acid liquor and the pulp are separated, the waste liquor being conducted from the blow pit by a conduit indicated conventionally at 3. From the blow pit the cellulose pulp is delivered to a treating tank indicated at 4, wherein it is subjected to reaction with an

alkaline liquor derived from the alkaline digestion of wood pulp. This alkaline digestion is carried on in a digester indicated at 5 wherein the wood chips are subjected to the action of an alkaline cooking liquor such as caustic soda or a solution containing caustic soda and sodium sulphide. When the caustic soda alone is employed as the cooking agent, the resulting cellulose product is commonly termed the soda pulp; but, when the alkaline cooking includes in addition to caustic soda a certain proportion of sodium sulphide, the cellulosic product resulting therefrom is commonly termed sulphate pulp or kraft pulp. After the pulp in digester 5 has been subjected to a cooking operation under high temperature and pressure for a sufficient length of time, the contents of the digester are delivered to a blow pit indicated at 6, from which both the pulp and the black liquor are delivered to a washer 7 in which the pulp is separated from the black liquor and is washed by the countercurrent system. I preferably employ a washer of the type shown in Letters Patent No. 1,421,664, dated July 4, 1922, in which a small amount of water is delivered to the washer by a pipe 8 at the same end of the washer from which the washed pulp is delivered. The black liquor is delivered from the washer through a conduit 9, and, as it is but slightly diluted by incoming wash water through conduit 8 and is at a high temperature, a portion thereof may be used in carrying on the digestion of the next batch of wood chips in digester 5. Consequently I have shown leading from the conduit 9 a conduit 10 by which a part of the black liquor is delivered to the upper end of digester 5 to be commingled with the fresh alkaline cooking liquor which is fed into the digester 5 after the chips have been placed therein. The black liquor emerging from the washer 7 is of a temperature of approximately from  $180^{\circ}$  to  $190^{\circ}$  F., and may have a free alkaline content of as high as 1%. I employ this black liquor, previous to the recovery of the soda content therefrom, in treating the pulp produced by the acid digestion and which as previously stated is collected in tank 4. Consequently the conduit 9 is connected with the tank 4 so as to deliver thereto the measured necessary volume to furnish the alkali necessary for the treatment of the pulp contained in 110

said tank. The purpose of treating the sulphite pulp contained in tank 4 is the removal of the greater portion of the less resistant cellulose,—the beta and gamma cellulose,—as well as the removal of lignin, resin and pentosan contained in the pulp. These materials are dissolved in the alkaline solution together with the greater portion of the less resistant cellulose. The presence 10 in the waste liquor of the organic constituents resulting from the previous alkaline digestion of the pulp in digester 5 does not interfere in any way with the dissolving and removal of the less resistant cellulose, 15 the lignin, the resin and the pentosan. The temperature of the waste alkaline black liquor is sufficient to cause the dissolving of the substances which I have mentioned, but, if desired, to speed the reaction, the tank 4 20 may be heated to a higher temperature by any suitable means. In some cases, it may be desirable to maintain the temperature of the alkaline solution at its boiling point. The tank 4 is also preferably provided with 25 agitating mechanism to ensure the thorough commingling of the hot black liquor with the pulp which is therein contained, and I have shown conventionally the tank as being provided with an agitator indicated at 30 25 for this purpose. After the pulp in the tank 4 has been subjected to hot alkaline treatment, it is now ready to be washed and recovered, but at the same time I desire also to recover the black liquor in order that 35 its valuable sodium compounds may be recovered for reuse in the production of an alkaline cooking liquor. For this purpose the pulp and alkaline liquor are drawn from the tank 4 and delivered to a washer 11 of the 40 counter-current type. This washer is of the same class as that indicated at 7 in which the pulp is delivered at one end of the instrumentality and the wash water at the other, and the two caused to pass in counter-current flow. A small amount of warm 45 water is fed to the washer through a pipe 12 and the contents of tank 4 are delivered to the other end of the washer by a conduit 13. The washed pulp, which is now characterized by a high alpha cellulose content and 50 a minimum proportion of beta and gamma cellulose, lignin, resin and pentosan, and which is also freed from the organic content of the black liquor by the washing operation, is delivered from the washer to tank 14. To this pulp may now be added 55 sufficient bisulphite antichlor to neutralize any residual traces of alkali that may remain in the pulp. The pulp, if desired, may 60 now be passed from the tank 14 through a conduit 15 to any suitable bleaching apparatus indicated conventionally at 16 for further bleaching and whitening of the pulp. The black liquor, together with the 65 small amount of wash water which is added

to the washer 11, is withdrawn from the washer through conduit 17 and is subjected to concentration and evaporation until it is of about the consistency of treacle. Inasmuch as there may be delivered from the alkaline digester a quantity of black liquor in excess of that needed for the alkaline treatment of the sulphite pulp, a portion of the black liquor from the washer 7 may be diverted from the conduit 9 and delivered 70 to the evaporator or concentrator together with the spent liquor from the washer 11. At 18 I have indicated conventionally a concentrating and evaporating apparatus which may be of the multiple-effect type. 75 The concentrated alkaline liquor, containing such organic compounds as were derived from the sulphite pulp, is now fed to a retort or furnace, and the soda content of the liquor is recovered therefrom in molten 80 condition. In the event that the alkaline liquor employed in the alkaline digestion is one comprising sodium sulphide, a reducing atmosphere may be maintained in the furnace or retort so as to recover the smelt 85 in the form of sodium carbonate and sodium sulphide; but, if the alkaline cooking liquor consists only of caustic soda, an oxidizing atmosphere may be maintained in the furnace so that the soda is recovered in the 90 form of sodium carbonate. Any additional make-up materials which may be needed, such as sodium sulphate or sodium carbonate, may be added to the evaporated 95 liquor before it is subjected to the smelting 100 operation.

At 19 I have indicated conventionally a furnace or retort and at 20 a dissolving tank into which the smelted sodium compounds are delivered from the furnace 19. 105 This tank contains an alkaline liquor in which the sodium compounds are dissolved. At 21 I have indicated the usual causticizing tank into which the solution from the dissolving tank is delivered, in which the liquor is causticized by the addition of a sufficient quantity of lime to react with the sodium carbonate and form caustic soda. At 22 I have indicated conventionally a filter press by which the calcium carbonate 110 resulting from the causticizing operation is filtered out from the liquor, the sludge being wasted or being recovered as desired and the filtrate being conducted by a conduit 23 to a storage tank 24 from which it is drawn as 115 needed for cooking wood chips in the alkaline digester 5.

Whereas I have shown only a single alkaline digester and a single sulphite digester, it will be of course understood that I may have any number of such digesters which will be blown in succession, so that the process which I have herein described is carried on continuously instead of intermittently. That is to say, the supply of pulp from the 120

digesters and the supply of black liquor from the alkaline digesters, by the use of such storage tanks as may be necessary, is such as to cause the operation of the washers 5 and the soda recovery furnace to be carried on continuously.

In addition to producing a pulp characterized by very high alpha cellulose content and a very low percentage of beta and 10 gamma cellulose, resin, lignin and pentosan, which itself is highly desirable,—the process which I have herein described is highly 15 advantageous in certain other respects, several of which may be mentioned. By utilizing a portion of the black liquor derived from the alkaline digestion in supplying the alkali necessary for treating the sulphite pulp, there is a marked conservation of 20 heat inasmuch as the black liquor delivered from the blow pit and the washer 7 is at a high temperature, so that but little heat is needed to maintain this or an even higher temperature in the digestion tank 4. Furthermore the alkali required in the digestion 25 of sulphite pulp does not represent a loss of chemical constituents inasmuch as this alkali is subsequently recovered. Moreover the liquor which is returned from the washer 11 has been enriched in organic constituents 30 which are combustible and which therefore increase the combustible characteristic of the original black liquor. Consequently, inasmuch as the black liquor which is now fed to the combustion retort has an increased

quantity of combustible matter, it allows a 35 more complete reduction of sodium sulphate in the event that it is desired to produce "sulphate" or kraft pulp.

What I claim is:

1. A process such as herein described, 40 which comprises treating sulphite pulp with alkaline black liquor resulting from the alkaline digestion of wood.

2. A process such as herein described, 45 which comprises treating sulphite pulp with alkaline black liquor resulting from the alkaline digestion of wood, separating such pulp from the alkaline liquor, and recovering the sodium components of said liquor.

3. A process such as herein described, 50 which comprises digesting wood with an alkaline cooking liquor, separating the hot waste liquor from the pulp, and treating sulphite pulp with such hot waste liquor.

4. A process such as herein described, 55 which comprises digesting wood with an alkaline cooking liquor, washing such pulp and separating the hot black liquor therefrom, treating sulphite pulp with said recovered hot alkaline black liquor, separating 60 the alkaline black liquor from such pulp, and concentrating and burning the combustible content of such black liquor and recovering the sodium components thereof.

In testimony whereof I have affixed my 65 signature.

GEORGE A. RICHTER.